

## UNITED STATES PATENT OFFICE

2,123,154

## DYEING OF TEXTILES

Erik Schirm, Dessau, Germany, assignor to General Aniline Works, Inc., New York, N. Y., a corporation of Delaware

No Drawing. Application July 11, 1933, Serial No. 679,890. In Germany July 12, 1932

4 Claims. (Cl. 8—5)

The direct dyeing of the vegetal as well as of the animal fibre with water-soluble dyestuffs is the simplest of all dyeing methods and at the same time the most harmless one for the fibre. 5 There is, however, the disadvantage of a more or less remarkable lack of fastness of the dyed materials to water and washing. Though there are in the prior art a great number of processes to overcome this deficiency, these processes take, 10 however, a certain constitution of the dyestuff for granted, their performance is in many cases rather complicated and none of them leads to a perfect washing-fastness such as is attainable by means of the vat-, sulphur- and ice-colours. 15 Now a process has been found which permits one to render more or less fast to washing any direct-dyeing performed on fibres of natural or regenerated cellulose. This process differs principally from the usual methods of increasing fastness in so far as the effect is not obtained by augmenting the molecule by adding water-insoluble residues to the dyestuff molecule, but by rendering ineffective the groups—in general sulpho- 20 or carboxyl groups—which bring about the water-solubility of the dyestuff and consequently its unfastness. This is obtained by forming salts which are absolutely insoluble and also resistant against the reaction of acids and alkalies as well as against soap. The quaternary ammonium bases 25 containing a system of no less than 8 non-interrupted conjugated double bonds, possessing substantive properties, have been recognized as eminently fit for the forming of such insoluble salts. These conjugated double bonds may be long either to open chains or to ring systems which may seem to be interrupted by imino groups in which cases I assume that, for instance, the group  $-\text{CO}-\text{NH}$  acts in the enolic form  $-\text{C}(\text{OH})=\text{N}-$ , so that really no interruption of 30 double linkings occurs. The new process consists therefore in the following: one begins with a direct dyeing on the fibre in the usual manner, whereupon the preliminarily dyed fibre is treated, with or without an intermediate rinsing, in a 35 second bath with the solution of a salt of the quaternary ammonium base which forms an insoluble salt; then one rinses, one soaps once more should it be necessary, one rinses again and finally one dries. If the dye is extracted completely or 40 almost completely from the dyeing bath, it is permissible to add directly to the exhausted dye bath also the ammonium base. It is not necessary that the quaternary ammonium base be colourless, but it may also be of a dyestuff character so that it is able to intensify the dying or to shade it off or to alter it completely.

This special embodiment of the present process offers the advantage that for the obtainment of a predetermined colour intensity one needs 45 only about half of the amount of acid or basic

dyestuffs in comparison with the amount required for an ordinary direct dyeing; in consequence of which the dyestuff is extracted from the bath relatively more intensively or even completely so that the aforementioned simple single-bath-procedure will be applicable. 5

From the experiments so far made it was discovered that substantive quaternary ammonium bases with at least two quaternary ammonium groups are particularly capable of making organic 10 compounds of an acid character fast to washing on the cellulose fibre.

The aforescribed after-treatment is of a prime importance for the mordant-drawing direct cotton dyestuffs because the dyed material 15 can thus be mordanted and rendered fast to washing in one and the same bath.

Further it has been stated, that it is also practicable to proceed inversely by treating the fibre first with the solution of the substantive quaternary ammonium base and after that with the dyestuff solution without its making any difference whether the ammonium base is colourless with the result that it serves so to speak merely as a mordant for the dyestuff to be laid upon, or 20 whether it also has colouring properties. Under certain circumstances it is not necessary that the dyestuff itself possesses any affinity for the fibre and the former will nevertheless be fixed upon the latter though it will not be fast to 25 washing. From this procedure there results the valuable practical procedure of tinging for instance the vegetal fibre after a preliminary treatment with a substantive, basic mordant of the above characterized sort, with so-called "acid 30 wool dyestuffs", which are not substantive or only to a little degree, while in many cases they 35 distinguish themselves from the really substantive dyestuffs by cheapness and higher fastness to light. 40

If the ammonium base be at the same time a dyestuff, it is not necessary that the acid component be likewise a dyestuff and it may therefore be represented by any higher molecular organic compound of an acid character, in which instance 45 it is the chief consideration that the latter forms an insoluble salt with the base. In certain cases it is advantageous if it possesses an affinity for the fibre such as is known for instance of certain sulphurized phenols. Substituted or non-substituted carbonic or sulphonic acids of the aliphatic, alicyclic, aromatic or fatty aromatic series are here likewise to be considered. Besides the dyeing effects it is possible to obtain at the same time a further refining effect consisting in rendering the textile goods supple, of a soft handle and of a water repelling property and with artificial silk one obtains certain matting effects, provided that as acid components one chooses soap forming carbonic or sulphonic acids, sulphonated fats 50 55 60

- and oils or higher molecular fatty alcohol sulphonates. Merely the latter refining effects are obtained if one combines a colourless, substantive ammonium base with the just named carbonic or sulphonic acids etc., whereby it is of course also practicable to replace part of the components by dyestuffs and thus to accomplish in one and the same operation the dying and the further refining.
- 10 As acid components one may also employ natural or artificial tanning principles, either alone or together with acid dyestuffs. In this case it is of a practical interest to employ natural tanning principles of the pyrogallol- or ellagene tannic acid category. It is already known that these tanning principles, by an after-treatment on the fibre with copper- and chromium salts, produce khaki-shades of an excellent fastness to light, while their fastness to washing can now be increased in the desired manner by adding the salt of a suitable substantive quaternary ammonium base in the same way as above described for mordant-drawing dyestuffs. As acid components there are finally to be considered the 20 above mentioned substantive compounds obtainable by sulphurizing of phenols and known for instance under the name of "katanoles".
- 25 It has already been suggested to render the direct dyeing on the fibre fast to water and 30 wet-ironing and in certain cases even fast to

and by combination of the thus formed mono-azo dyestuff in alkaline solution with 1 molecule of diazotized tolusafranine (Schultz-Julius, I. c. Nr. 679). Then one heats up to 95-100° C. and keeps this temperature for 25 to 30 minutes, whereupon one rinses and dries. As a result a very good black dyeing fast to washing is obtained.

#### Example 3

Cotton is dyed under usual conditions with 1% of benzo-light-blue FR (cf. Fierz-David, Grundlegende Operationen der Farbenchemie, 1922, p. 147) from a neutral bath containing common salt. The dyestuff having completely been drawn on the fibre, one adds immediately and in the form of a hot concentrated solution 1,5% of the reddish blue, substantive dyestuff prepared by diazotizing and coupling of 2 molecules of tolusafranine with 1 molecule of  $\alpha$ -naphthol; the bath is kept at boiling temperature until the second dyestuff is likewise drawn on entirely or almost entirely, whereupon one rinses and dries. The thus obtained blackblue dyeing is of an excellent fastness to washing and light.

#### Example 4

Cotton or viscose-artificial silk is worked for 45 minutes and at 85-100° C. in a bath which in a bath-length of 1:15 contains 2% of an ammonium salt of the following constitution:



- 35 after-dyeing by an after-treatment with amines or ammonium bases containing a high molecular fatty acid residue. This process produces, however, no fastness to washing and merely a quite imperfect improvement.

#### Example 1

- 40 A 2% dyeing of Congo-red performed in the usual manner on cotton, is rinsed and wrung out, then it is treated for half an hour at 90-100° C. in a bath containing 1 g. per liter of the 45 methylsulphuric salt of a substantive disazoammonium base of the following constitution:



- 50 whereupon it is taken out, rinsed and dried. The thus obtained tone which compared with the original dyeing shows a more yellowish shade, shows an excellent fastness to washing when 55 treated for half an hour in a 0.2% soap solution at 90-100° C., whereas the original dyeing will under the same conditions heavily bleed out into the soap bath and in a great part is drawn off from the fibre.

- 60 The above mentioned base is obtained by coupling tetrazotized benzidine with dimethylaniline and addition of dimethylsulphate to the azo-dye-stuff in a nitrobenzol-solution at about 120-150° C. The methylsulphuric salt is yellow, very easily 65 soluble in water and hygroscopic.

#### Example 2

- 70 One makes next in the usual manner a 2% dyeing of direct-darkblack EW (Schultz-Julius, Farbstofftabellen 1914, Nr. 462) on cotton, then one rinses, whereupon the material is brought in wet state and at a temperature at about 40° C. into a bath containing 2% of a substantive basic dyestuff, obtainable by acid coupling of 1 molecule of diazotized trimethyl-m-aminophenylammonium chloride with 1 molecule of  $\alpha$ -naphthol

35 further 5% of acetic acid and 20% of common salt. Then one washes cold, whereupon the material while moist is brought into a dyeing bath at a temperature of 60° C. containing 1% of Orange II (Schultz-Julius, I. c. Nr. 145) or of another acid wool dyestuff and 20% of common salt in a bath-length of 1:20. The dyeing bath will be exhausted in a short time.

The above substantive ammonium base can be obtained in the following manner: p-aminodimethyl-aniline is condensed in pyridine solution with 1 mol. of p-nitrobenzoyl chloride. Dimethylsulphate is added to the condensation product



50 whereupon one reduces the nitro group to the amino group and the thus obtained intermediate product is condensed with chloride of cinnamic acid in presence of acid binding stuffs. It is also practicable and advantageous to condense 55 2 mols of the intermediate product by means of 1 mol. of phosgene or terephthaloylchloride in a pyridine solution.

If one substitutes a substantive basic dyestuff with one or more quaternary ammonium groups (cf. e. g. the German Patents 93,499 and 97,244) for the substantive ammonium base, one obtains the practicability of producing many different colour tones in combining both colours of the basic and of the acid dyestuff (cf. the following example).

If one chooses as acid dyestuff an after-chromatable one, the after-chromating can be done in a third bath or immediately in the acid dyeing bath.

#### Example 5

Cotton or viscose silk is brought at about 60° C. into a dyeing bath (bath-length 1:10 to 1:15), containing 2% of a substantive, basic dyestuff obtainable by the coupling of 2 mols of diazo-

5

10

15

20

25

30

35

40

45

50

55

60

65

70

75

tized chloride of trimethyl-(m-aminophenyl)-ammonium with 1 mol. of bis-(2',3'-oxynaphthoyl-) benzidine in an alcoholic-alkaline solution. One dyes for 1 hour at 90-100° C. in adding 5 2% of acetic acid and 20% of common salt, then one cools down and rinses, whereupon the material is brought into a bath containing 2% of Congo-red in a bath-length of 1:15, wherein it is worked for about half an hour at boiling temperature. After that the bath will be nearly exhausted and one can rinse and dry. There results a bluish-red dyeing which is very fast to washing.

*Example 6*

15 Cotton is worked for 1 hour at 85° C. in a bath (in a bath-length of 1:15) containing 1% of the compound according to the following formula:



further 1% of soda and 20% of sodium sulphate. Then one rinses cold, whereupon an after-treatment of half an hour takes place in a warm bath of 1% of the disazo dyestuff of tetrazotized 30 benzidine and 2-oxynaphthyl-7-trimethylammonium chloride (cf. German Patent 90,310), 2% of acetic acid and 10% of common salt.

The above "acid and substantive mordant" is obtainable by condensing 1,5-naphthylene-diamine-3,7-disulphonic acid sodium with the chloride of cinnamic acid in presence of an acid binding agent. It may be replaced with good results by the products which are obtained by the sulphurizing of phenols ("katanol").

*Example 7*

40 1% of the dyestuff obtainable by the coupling of tetrazotized dianisidine with 2-oxynaphthyl-7-trimethyl-ammonium chloride (cf. German Patent 90,310) jointly with 4% of the "substantive basic mordants" mentioned in Example 4, is dyed on cotton or viscose silk as indicated therein. An after-treatment takes place in a hot bath containing 2 g. of sodium laurylsulphonate per litre. The thus dyed material is of a soft and 50 agreeable handle.

Instead of the sodium lauryl-sulphonate one can likewise apply sodium cetyl- or octadecylsulphonate or Turkey red oil or the sulphuric acid ester salts of the dodecyl-, tetradecyl-, cetyl- or 55 octadecyl-alcohol or compounds with similar properties such as oleyltaurin.

60

*Example 8*

65 One proceeds exactly as stated in Example 3 with the exception of employing diamine-brown M (Schultz-Julius, 1. c. Nr. 344) as acid direct dyestuff. The violetblackish combination-dyeing which is already rather fast to washing, has an after-treatment to undergo for 25 minutes at 80-100° C. in a development bath with 1.5% of acetic acid, 1.5% of bichromate of potassium and 70 1.5% of copper vitriol in a bath-length of 1:15. The dyeing is then of a dark bluishblack and eminently fast to washing and light.

*Example 9*

75 Cotton cloth is worked for 1 hour at 85° C. with

10% of a tannin extract of the pyrogallol- or ellagene tannic acid category such as myrobalan-, dividivi- or mango-leaves extract, in a bath-length of 1:15. Then one squeezes off and without an intermediate rinsing, the material is brought into a development bath at 60° C. containing 5 2.5% of the disazoammonium base as per Example 1, in a bath-length of 1:15. After digesting at 80-100° C. until the ammonium base is completely taken up one adds 2.5% of sodium bichromate and 2.5% of copper vitriol, then one gently agitates for 20 minutes at 80-90° C., whereupon one cools and rinses. There results a khaki-dyeing of an excellent fastness to light and washing.

*Example 10*

20 3% of the dyestuff employed in Example 3 composed of diazotized tolusafranine and  $\alpha$ -naphthol are dyed on cotton while boiling for about  $\frac{3}{4}$  of an hour and with an addition of 3% of acetic acid and 20% of common salt. Then one cools down to about 40° C. under continuous agitation, at this temperature one adds 10% of tannin extract (myrobalan, dividivi, mango leaves extract) dissolved in a small amount of hot water, whereupon one heats to obtain re-boiling. After about half an hour one takes the cotton out of the bath and develops the dyeing for 25-30 minutes at 80-100° C. in a fresh bath containing 2% of bichromate of potassium, 2% of acetic acid and 2% of copper sulphate in a bath-length of 1:20. There results a dark bluish-black dyeing of an excellent fastness to washing and light.

25 What I claim is:

30 1. A process for dyeing cellulosic fibers which comprises producing on the fiber an insoluble salt of a substantive dyestuff and a substantive quaternary ammonium base containing at least two quaternary ammonium groups and a system of no less than 8 conjugated non-interrupted double linkings in its molecule, whereby dyeings fast to washing are obtained.

35 2. A process for dyeing cellulosic fibers which comprises dyeing the fiber by means of a substantive dyestuff and after-treating the dyeing thus obtained with the solution of a substantive quaternary ammonium base containing at least two quaternary ammonium groups and a system of no less than 8 conjugated non-interrupted double linkings in its molecule, whereby dyeings fast to washing are obtained.

40 3. A process for dyeing cellulosic fibers which comprises dyeing the fiber by means of a substantive dyestuff and after-treating the dyeing thus obtained with the solution of a substantive disazonium base of the formula:



45 whereby dyeings fast to washing are obtained.

55 4. The process for dyeing cellulosic fibres which comprises dyeing the fibre by means of a substantive dye-stuff and after-treating the dyeing thus obtained with the solution of an ammonium salt of the formula:



70 whereby dyeings fast to washing are obtained.